

## UNITED STATES PATENT OFFICE.

MICHAEL G. MINAEFF, OF BROOKLYN, AND ALBERT PARSONS SACHS, OF NEW YORK, N. Y., ASSIGNEES, BY MESNE ASSIGNMENTS, TO THE LARVEX CORPORATION, OF BROOKLYN, NEW YORK, A CORPORATION OF NEW YORK.

## MOTHPROOFED ARTICLE.

No Drawing.

Application filed July 17, 1925. Serial No. 44,363.

This invention pertains to articles, more especially articles composed of wool or other animal fibers, in whole or in part, which possess certain novel chemical and physical characteristics which have been imparted to them by treatment with special moth proofing preventive compositions. Among the specific materials embraced within the invention may be mentioned yarn, fiber, hair or similar animal fibers, and the articles made therefrom, such as fabrics and piece goods of various kinds, furs, tissue, or other forms of associated or massed fibers. 5 The materials specified, having been treated as hereinafter described, are resistant to the attack of moth larvæ without substantial diminution in their tensile strengths or deterioration in any other respect, are substantially neutral in character and normal to the feel, and have adsorbed in the fibers thereof certain compounds of fluorine, aluminum and silicon. The presence of these elements is revealed by suitable analytical 20 chemical tests well known to the art.

Typical of a specific moth proofing composition which we may employ in producing the novel articles or products specified is the following:

|                        | Per cent. |
|------------------------|-----------|
| Sodium silico fluoride | 0.5       |
| Alum                   | 0.3       |
| Oxalic or citric acid  | 0.01      |

It will be noted that an especially small percentage of the organic acid is employed, in contradistinction to the strong acid solutions of the prior art which act detrimentally on fibers. The relatively small amount herein employed has no detrimental action on the fibers, but is advantageous in that it serves to enhance the permanency of the immunity to the moth larvæ.

The materials to be moth proofed are either dipped into an aqueous solution containing the above ingredients, preferably in the proportions specified, or the materials may be sprayed with the solution. Regardless of the specific method of treatment, assuming the solution is properly adsorbed by the fibers, the ultimate articles possess

the characteristics enumerated above. It is probable that there may be an interaction between or among the ingredients, entering into the composition, but, in any event, the chemical qualities enumerated, namely, the presence of fluorine, aluminum and silicon characterizes the treated materials.

The scope of the invention is commensurate with the appended claims.

Having thus fully described the invention, what we claim as new and desire to secure by Letters Patent is:

1. As a new article of manufacture, animal fibers impregnated with a moth repellent composition resulting from a mixture of compounds of fluorine, silicon and aluminum.
2. As a new article of manufacture, animal fibers impregnated with a moth repellent composition comprising water soluble compounds of fluorine, silicon and aluminum.
3. As a new article of manufacture, fibrous material wherein the constituent fibers are impregnated with a moth resistant composition containing a water soluble silico fluoride and a water soluble aluminum salt.
4. As a new article of manufacture, fibrous material wherein the constituent fibers are impregnated with a moth resistant composition containing sodium silico fluoride and alum.
5. As a new article of manufacture, fibrous material wherein the constituent fibers are impregnated with a moth resistant composition containing sodium silico fluoride, alum, and a small quantity of an organic acid.
6. A new article of manufacture embodying animal fibers which have been rendered moth proof by a composition containing a water soluble compound of fluorine and silicon and a water soluble salt of aluminum, said fibers being substantially neutral chemically and not deteriorated by the process of moth proofing.
7. A new article of manufacture embodying animal fibers which have been rendered moth proof by an impregnation of their fibers with a solution containing a

water soluble compound of fluorine and silicon, and a water soluble salt of aluminum, said solution being allowed to dry thereon without washing or further treatment.

8. A moth repellent fiber having incorporated therein the products resulting from

the aqueous interaction of sodium silico fluoride and water soluble aluminum salts. In testimony whereof we have signed the foregoing specification.

MICHAEL G. MINAEFF.  
ALBERT PARSONS SACHS.